



US01079976B2

(12) **United States Patent**  
**Takubo et al.**

(10) **Patent No.:** **US 10,799,766 B2**  
(b4) **Date of Patent:** **Oct. 13, 2020**

(54) **GOLF BALL**

(71) Applicant: **SUMITOMO RUBBER INDUSTRIES, LTD.**, Kobe-shi, Hyogo (JP)

(72) Inventors: **Toshiyuki Takubo**, Kobe (JP); **Takahiro Sajima**, Kobe (JP)

(73) Assignee: **SUMITOMO RUBBER INDUSTRIES, LTD.**, Kobe-Shi, Hyogo (JP)

(\*) Notice: Subject to any disclaimer, the term of this patent is extended or adjusted under 35 U.S.C. 154(b) by 0 days.

(21) Appl. No.: **16/209,494**

(22) Filed: **Dec. 4, 2018**

(65) **Prior Publication Data**

US 2019/0192921 A1 Jun. 27, 2019

(30) **Foreign Application Priority Data**

Dec. 26, 2017 (JP) ..... 2017-249523

(51) **Int. Cl.**

*A63B 37/12* (2006.01)  
*A63B 37/14* (2006.01)  
*A63B 37/06* (2006.01)  
*A63B 37/00* (2006.01)  
*A63B 1/00* (2006.01)

(52) **U.S. Cl.**

CPC ..... *A63B 37/0074* (2013.01); *A63B 1/00* (2013.01); *A63B 37/0006* (2013.01); *A63B 37/008* (2013.01); *A63B 37/0083* (2013.01); *A63B 37/0092* (2013.01)

(58) **Field of Classification Search**

USPC ..... 473/351-385  
See application file for complete search history.

## (56)

**References Cited**

## U.S. PATENT DOCUMENTS

5,704,852 A \* 1/1998 Kato ..... A63B 37/0003  
473/357  
5,722,903 A \* 3/1998 Moriyama ..... A63B 37/0004  
40/327  
6,089,847 A \* 7/2000 Inoue ..... B29C 45/14073  
264/278  
6,129,881 A \* 10/2000 Puniello ..... B29C 45/14073  
264/102  
6,238,194 B1 \* 5/2001 Inoue ..... B29C 45/14073  
264/278  
6,561,929 B2 \* 5/2003 Watanabe ..... A63B 37/0003  
473/377  
6,815,507 B2 \* 11/2004 Ohama ..... A63B 37/0003  
473/371

(Continued)

## FOREIGN PATENT DOCUMENTS

JP 2017-108862 A 6/2017

*Primary Examiner* — Alvin A Hunter

(74) *Attorney, Agent, or Firm* — Birch, Stewart, Kolasch & Birch, LLP

(57) **ABSTRACT**

A golf ball 2 includes a core 4 and a cover 6 positioned outside the core 4. The cover 6 is molded in a mold having support pins by injection molding. A ratio (K/S) of a surface hardness K of the core 4 to an amount of compressive deformation S of the core 4 satisfies the following mathematical formula.

$$13.0 \leq K/S \leq 24.0$$

The cover 6 has a hardness H of not greater than 62. A product ( $\alpha^*V$ ) of a latitude  $\alpha$  of each support pin and a volume V of the cover 6 is not less than 300.

**5 Claims, 11 Drawing Sheets**

2



(56)

**References Cited**

U.S. PATENT DOCUMENTS

- 7,153,467 B2 \* 12/2006 Brum ..... A63B 37/0003  
264/553  
7,201,674 B2 \* 4/2007 Ohama ..... A63B 37/0003  
473/383  
7,381,041 B2 \* 6/2008 Wilber ..... B29C 33/44  
425/116  
7,390,273 B2 \* 6/2008 Ohama ..... A63B 37/0003  
473/383  
7,704,431 B2 \* 4/2010 Endo ..... B29C 45/14073  
264/275  
7,718,107 B2 \* 5/2010 Endo ..... B29C 45/14073  
264/259  
7,727,437 B2 \* 6/2010 Higuchi ..... B29C 45/0055  
264/162  
8,388,466 B2 \* 3/2013 Ohama ..... A63B 37/0003  
473/377  
8,388,882 B2 \* 3/2013 Omura ..... A63B 37/0003  
249/115  
8,512,619 B2 \* 8/2013 Tutmark ..... B29C 33/123  
264/278  
8,662,882 B2 \* 3/2014 Wang ..... B29C 45/2708  
425/573  
8,882,490 B2 \* 11/2014 Felker ..... B29C 45/0025  
425/542  
9,149,687 B2 \* 10/2015 Okabe ..... C08G 63/47  
9,278,467 B2 \* 3/2016 Nakagawa ..... B29C 45/14819  
2017/0173400 A1 6/2017 Sajima et al.

\* cited by examiner



Fig. 1



Fig. 2



Fig 3

2



Fig. 4



Fig. 5



Fig. 6



Fig. 7



Fig. 8



Fig. 9



Fig. 10



Fig. 11



Fig. 12



Fig. 13



Fig. 14



Fig. 15



Fig. 16

# 1

## GOLF BALL

This application claims priority on Patent Application No. 2017-249523 filed in JAPAN on Dec. 26, 2017. The entire contents of this Japanese Patent Application are hereby incorporated by reference.

### BACKGROUND OF THE INVENTION

#### Field of the Invention

The present invention relates to golf balls. Specifically, the present invention relates to golf balls having a core and a cover.

#### Description of the Related Art

In an accurate shot, a golf ball is hit at the sweet spot of a clubface. The shock generated upon this shot is small. Upon a mishit, a golf ball is hit at a location other than the sweet spot of a clubface. The shock upon a mishit is great. The great shock gives pain to the hands of the golf player. At this time, the golf player feels discomfort. In particular, upon a mishit made when the air temperature is low (for example, in winter), the golf player feels acute pain.

Generally, golf players desire golf balls having favorable feel at impact. In particular, beginners prefer golf balls having soft feel at impact. This is because the frequency of mishits is high in play by beginners.

Furthermore, golf players also place importance on feel at impact upon putting. Generally, golf players desire golf balls with which soft feel at impact is obtained upon putting.

So-called thread-wound balls used to be mainstream golf balls. At present, thread-wound balls are almost not commercially available. In golf in recent years, so-called solid golf balls such as two-piece balls, three-piece balls, four-piece balls, five-piece balls, six-piece balls, and the like are used.

A solid golf ball has a solid core and a cover. The cover of this golf ball can be molded by injection molding. Therefore, this golf ball can be produced at low cost. In injection molding, the core is held at the center of the cavity of a mold. A melted resin composition is injected into the space between the core and the cavity face. The resin composition is solidified, whereby the cover is molded. A proposal concerning a two-piece ball, which is one type of solid golf ball, is disclosed in JP2017-108862.

Upon shots with drivers by beginners, golf balls often fly in unintended directions. Golf balls often fall into a pond or fly into the woods. Beginners often lose golf balls. Therefore, beginners do not prefer expensive golf balls. Solid golf balls are suitable for beginners, since solid golf balls can be produced at low cost.

As described above, beginners prefer soft feel at impact upon shots and upon putting. Improvement of feel at impact of solid golf balls is desired.

With a solid golf ball in which a cover having a small volume is used, soft feel at impact can be achieved upon shots and upon putting. In molding this cover, the space between the core and the cavity face is small. The small space causes a failure of injection of the melted resin composition.

With a golf ball in which a core having a large amount of compressive deformation is used, the core significantly deforms upon a shot with a driver. This deformation can contribute to soft feel at impact upon the shot with the driver. However, in molding the cover of this golf ball, the core

# 2

significantly deforms by injection pressure. The core is locally radially enlarged, so that the space between the core and the cavity face is locally reduced. This reduction causes a local failure of injection of the melted resin composition. In particular, a failure of injection is likely to occur near each pole.

In injection molding, a core is held by a plurality of support pins. Each support pin is located near the pole. When the core is sufficiently pressed by the support pins, the core is inhibited from being radially enlarged near each pole.

With a golf ball in which a core having a low surface hardness is used, soft feel at impact can be achieved upon putting. However, since the surface hardness of the core is low, pressing of the core by each support pin is likely to be concentrated only in the vicinity of the leading end of the support pin. The core is still locally and radially enlarged near the pole and at a location slightly away from the support pin, on the surface of the core. Regarding the golf ball in which the core having a low surface hardness is used, a failure of injection is likely to occur near each pole during molding of the cover.

An object of the present invention is to provide a golf ball having excellent feel at impact upon a shot with a driver and excellent feel at impact upon putting, and having excellent cover moldability.

### SUMMARY OF THE INVENTION

A golf ball according to the present invention includes a core and a cover positioned outside the core and molded in a mold having a plurality of support pins by injection molding. A ratio (K/S) of a surface hardness K (Shore C) of the core to an amount of compressive deformation S (mm) of the core satisfies the following mathematical formula.

$$13.0 \leq K/S \leq 24.0$$

The cover has a hardness H (Shore D) of not greater than 62. The golf ball has a plurality of dimples on a surface thereof. A total volume W of the dimples is not less than 490 mm<sup>3</sup> and not greater than 620 mm<sup>3</sup>. A product ( $\alpha^*V$ ) of a latitude  $\alpha$  (degree) of each support pin and a volume V (cm<sup>3</sup>) of the cover is not less than 300.

Since the ratio (K/S), the hardness H of the cover, and the product ( $\alpha^*V$ ) are appropriate, the golf ball according to the present invention has excellent feel at impact upon a shot with a driver, excellent feel at impact upon putting, and excellent cover moldability.

Preferably, the amount of compressive deformation S of the core is not less than 3.5 mm. Preferably, a number of the support pins is not less than 8 and not greater than 12. Preferably, a number of the dimples is not less than 300 and not greater than 400. Preferably, the golf ball has a two-piece structure.

According to another aspect, a method for producing a golf ball according to the present invention includes the steps of:

placing a core into a mold having a plurality of support pins and having a cavity face including a plurality of pimples;

holding the core in a cavity of the mold by the support pins;

injecting a melted resin composition into a space between the cavity face and the core; and

solidifying the resin composition to mold a cover and form a plurality of dimples having a shape that is an inverted shape of the pimples.

In the golf ball obtained by this production method, a ratio (K/S) of a surface hardness K (Shore C) of the core to an amount of compressive deformation S (mm) of the core satisfies the following mathematical formula.

$$13.0 \leq K/S \leq 24.0$$

The cover of the golf ball has a Shore D hardness of not greater than 62. A total volume W of the dimples is not less than 490 mm<sup>3</sup> and not greater than 620 mm<sup>3</sup>. A product ( $\alpha^*V$ ) of a latitude  $\alpha$  (degree) of each support pin and a volume V (cm<sup>3</sup>) of the cover is not less than 300.

#### BRIEF DESCRIPTION OF THE DRAWINGS

FIG. 1 is a cross-sectional view of a golf ball according to an embodiment of the present invention;

FIG. 2 is a plan view of the golf ball in FIG. 1;

FIG. 3 is a front view of the golf ball in FIG. 2;

FIG. 4 is a partially enlarged cross-sectional view of the golf ball in FIG. 1;

FIG. 5 is a cross-sectional view of a mold for the golf ball in FIG. 1, with a core of the golf ball;

FIG. 6 is a cross-sectional view of the mold in FIG. 5, with the core and a cover;

FIG. 7 is a partially enlarged view of the mold in FIG. 6, with the core and the cover.

FIG. 8 is a partially enlarged view of a support pin of the mold in FIG. 7;

FIG. 9 is a plan view of a golf ball according to Example 8 of the present invention;

FIG. 10 is a front view of the golf ball in FIG. 9;

FIG. 11 is a plan view of a golf ball according to Example 7 of the present invention;

FIG. 12 is a front view of the golf ball in FIG. 11;

FIG. 13 is a plan view of a golf ball according to Example 6 of the present invention;

FIG. 14 is a front view of the golf ball in FIG. 13;

FIG. 15 is a plan view of a golf ball according to Comparative Example 3; and

FIG. 16 is a front view of the golf ball in FIG. 15.

#### DESCRIPTION OF THE PREFERRED EMBODIMENTS

The following will describe in detail the present invention based on preferred embodiments with appropriate reference to the drawings.

A golf ball 2 shown in FIG. 1 includes a spherical core 4 and a cover 6 positioned outside the core 4. In this embodiment, the cover 6 is directly joined to the core 4. The golf ball 2 is a so-called two-piece ball. The golf ball 2 has a plurality of dimples 8 on the surface thereof. Of the surface of the golf ball 2, a part other than the dimples 8 is a land 10. The golf ball 2 includes a paint layer and a mark layer on the external side of the cover 6 although these layers are not shown in the drawing.

The core 4 may include two or more layers. In this case, each layer may be formed from a rubber composition or may be formed from a resin composition. The cover 6 is the outermost layer excluding the paint layer and the mark layer.

The golf ball 2 preferably has a diameter of not less than 40 mm and not greater than 45 mm. From the viewpoint of conformity to the rules established by the United States Golf Association (USGA), the diameter is particularly preferably not less than 42.67 mm. In light of suppression of air

resistance, the diameter is more preferably not greater than 44 mm and particularly preferably not greater than 42.80 mm.

The golf ball 2 preferably has a weight of not less than 40 g and not greater than 50 g. In light of attainment of great inertia, the weight is more preferably not less than 44 g and particularly preferably not less than 45.00 g. From the viewpoint of conformity to the rules established by the USGA, the weight is particularly preferably not greater than 45.93 g.

The core 4 is formed by crosslinking a rubber composition. Examples of preferable base rubbers for use in the rubber composition include polybutadienes, polyisoprenes, styrene-butadiene copolymers, ethylene-propylene-diene copolymers, and natural rubbers. In light of resilience performance, polybutadienes are preferable. When a polybutadiene and another rubber are used in combination, it is preferred if the polybutadiene is a principal component. Specifically, the proportion of the polybutadiene to the entire base rubber is preferably not less than 50% by weight and particularly preferably not less than 80% by weight. A polybutadiene in which the proportion of cis-1,4 bonds is not less than 80% is particularly preferable.

The rubber composition of the core 4 preferably includes a co-crosslinking agent. Preferable co-crosslinking agents in light of durability and resilience performance of the golf ball 2 are monovalent or bivalent metal salts of an  $\alpha,\beta$ -unsaturated carboxylic acid having 2 to 8 carbon atoms. Examples of preferable co-crosslinking agents include zinc acrylate, magnesium acrylate, zinc methacrylate, and magnesium methacrylate. In light of durability and resilience performance of the golf ball 2, zinc acrylate and zinc methacrylate are particularly preferable.

The rubber composition may include a metal oxide and an  $\alpha,\beta$ -unsaturated carboxylic acid having 2 to 8 carbon atoms. They both react with each other in the rubber composition to obtain a salt. The salt serves as a co-crosslinking agent. Examples of preferable  $\alpha,\beta$ -unsaturated carboxylic acids include acrylic acid and methacrylic acid. Examples of preferable metal oxides include zinc oxide and magnesium oxide.

The amount of the co-crosslinking agent per 100 parts by weight of the base rubber is preferably not less than 10 parts by weight. Deformation of the core 4 in which this amount is not less than 10 parts by weight is small during molding of the cover 6. The core 4 can contribute to the moldability of the golf ball 2. The golf ball 2 having the core 4 also has excellent resilience performance. From these viewpoints, this amount is more preferably not less than 15 parts by weight and particularly preferably not less than 20 parts by weight.

The amount of the co-crosslinking agent per 100 parts by weight of the base rubber is preferably not greater than 40 parts by weight. The core 4 in which this amount is not greater than 40 parts by weight sufficiently deforms when the golf ball 2 is hit with a driver. The core 4 can achieve soft feel at impact for the golf ball 2 upon a shot with a driver. With the golf ball 2 having the core 4, soft feel at impact can also be achieved upon putting. From these viewpoints, this amount is more preferably not greater than 35 parts by weight and particularly preferably not greater than 30 parts by weight.

Preferably, the rubber composition of the core 4 includes an organic peroxide. The organic peroxide serves as a crosslinking initiator. The organic peroxide contributes to the durability and the resilience performance of the golf ball 2. Examples of suitable organic peroxides include dicumyl

peroxide, 1,1-bis(t-butylperoxy)-3,3,5-trimethylcyclohexane, 2,5-dimethyl-2,5-di(t-butylperoxy)hexane, and di-t-butyl peroxide. An organic peroxide with particularly high versatility is dicumyl peroxide.

The amount of the organic peroxide per 100 parts by weight of the base rubber is preferably not less than 0.1 parts by weight. Deformation of the core 4 in which this amount is not less than 0.1 parts by weight is small during molding of the cover 6. The core 4 can contribute to the moldability of the golf ball 2. The golf ball 2 having the core 4 also has excellent resilience performance. From these viewpoints, this amount is more preferably not less than 0.3 parts by weight and particularly preferably not less than 0.5 parts by weight.

The amount of the organic peroxide per 100 parts by weight of the base rubber is preferably not greater than 3.0 parts by weight. The core 4 in which this amount is not greater than 3.0 parts by weight sufficiently deforms when the golf ball 2 is hit with a driver. The core 4 can achieve soft feel at impact for the golf ball 2 upon a shot with a driver. With the golf ball 2 having the core 4, soft feel at impact can also be achieved upon putting. From these viewpoints, this amount is more preferably not greater than 2.5 parts by weight and particularly preferably not greater than 2.0 parts by weight.

Preferably, the rubber composition of the core 4 includes an organic sulfur compound. Organic sulfur compounds include naphthalenethiol compounds, benzenethiol compounds, and disulfide compounds.

Examples of naphthalenethiol compounds include 1-naphthalenethiol, 2-naphthalenethiol, 4-chloro-1-naphthalenethiol, 4-bromo-1-naphthalenethiol, 1-chloro-2-naphthalenethiol, 1-bromo-2-naphthalenethiol, 1-fluoro-2-naphthalenethiol, 1-cyano-2-naphthalenethiol, and 1-acetyl-2-naphthalenethiol.

Examples of benzenethiol compounds include benzenethiol, 4-chlorobenzenethiol, 3-chlorobenzenethiol, 4-bromobenzenethiol, 3-bromobenzenethiol, 4-fluorobenzenethiol, 4-iodobenzenethiol, 2,5-dichlorobenzenethiol, 3,5-dichlorobenzenethiol, 2,6-dichlorobenzenethiol, 2,5-dibromobenzenethiol, 3,5-dibromobenzenethiol, 2-chloro-5-bromobenzenethiol, 2,4,6-trichlorobenzenethiol, 2,3,4,5,6-pentachlorobenzenethiol, 2,3,4,5,6-pentafluorobenzenethiol, 4-cyanobenzenethiol, 2-cyanobenzenethiol, 4-nitrobenzenethiol, and 2-nitrobenzenethiol.

Examples of disulfide compounds include diphenyl disulfide, bis(4-chlorophenyl)disulfide, bis(3-chlorophenyl)disulfide, bis(4-bromophenyl)disulfide, bis(3-bromophenyl)disulfide, bis(4-fluorophenyl)disulfide, bis(4-iodophenyl)disulfide, bis(4-cyanophenyl)disulfide, bis(2,5-dichlorophenyl)disulfide, bis(3,5-dichlorophenyl)disulfide, bis(2,6-dichlorophenyl)disulfide, bis(2,5-dibromophenyl)disulfide, bis(3,5-dibromophenyl)disulfide, bis(2-chloro-5-bromophenyl)disulfide, bis(2-cyano-5-bromophenyl)disulfide, bis(2,4,6-trichlorophenyl)disulfide, bis(2-cyano-4-chloro-6-bromophenyl)disulfide, bis(2,3,5,6-tetrachlorophenyl)disulfide, bis(2,3,4,5,6-pentachlorophenyl)disulfide, and bis(2,3,4,5,6-pentabromophenyl)disulfide.

In light of resilience performance of the golf ball 2, the amount of the organic sulfur compound per 100 parts by weight of the base rubber is preferably not less than 0.1 parts by weight and particularly preferably not less than 0.2 parts by weight. In light of soft feel at impact upon a shot with a driver and upon putting, the amount is preferably not greater than 1.5 parts by weight, more preferably not greater than

1.0 parts by weight, and particularly preferably not greater than 0.8 parts by weight. Two or more organic sulfur compounds may be used in combination.

The rubber composition of the core 4 may include a filler for the purpose of specific gravity adjustment and the like. Examples of suitable fillers include zinc oxide, barium sulfate, calcium carbonate, and magnesium carbonate. The amount of the filler is determined as appropriate so that the intended specific gravity of the core 4 is accomplished.

The rubber composition of the core 4 may include a carboxylic acid or a carboxylate. The core 4 including a carboxylic acid or a carboxylate has a low hardness around the central point thereof. The core 4 has an outer-hard/inner-soft structure. When the golf ball 2 including the core 4 is hit with a driver, the spin rate is low. With the golf ball 2 having a low spin rate, a large flight distance is obtained. Examples of preferable carboxylic acids include benzoic acid. Examples of preferable carboxylates include zinc octoate and zinc stearate. The rubber composition particularly preferably includes benzoic acid. The total amount of the carboxylic acid and the carboxylate per 100 parts by weight of the base rubber is preferably not less than 1 part by weight and not greater than 20 parts by weight.

The rubber composition may include various additives, such as sulfur, an anti-aging agent, a coloring agent, a plasticizer, a dispersant, and the like, in an adequate amount. The rubber composition may include crosslinked rubber powder or synthetic resin powder.

The core 4 preferably has a diameter of not less than 39.0 mm. In the golf ball 2 having the core 4 having a diameter of not less than 39.0 mm, the cover 6 is thin. Therefore, the golf ball 2 has excellent feel at impact. Furthermore, the golf ball 2 has excellent resilience performance. From these viewpoints, the diameter is more preferably not less than 39.3 mm and particularly preferably not less than 39.8 mm. In light of moldability and durability of the golf ball 2, the diameter is preferably not greater than 42.0 mm, more preferably not greater than 41.5 mm, and particularly preferably not greater than 41.1 mm.

The core 4 preferably has an amount of compressive deformation S of not less than 3.5 mm. The core 4 having an amount of compressive deformation S of not less than 3.5 mm sufficiently deforms when the golf ball 2 is hit with a driver. The core 4 can achieve soft feel at impact for the golf ball 2. From this viewpoint, the amount of compressive deformation S is more preferably not less than 3.8 mm and particularly preferably not less than 4.0 mm.

The amount of compressive deformation S is preferably not greater than 6.0 mm. Deformation of the core 4 having an amount of compressive deformation S of not greater than 6.0 mm is small during molding of the cover 6. The core 4 can contribute to the moldability of the golf ball 2. The golf ball 2 having the core 4 also has excellent resilience performance. From these viewpoints, the amount of compressive deformation S is more preferably not greater than 5.7 mm and particularly preferably not greater than 5.5 mm.

For measurement of the amount of compressive deformation S, a YAMADA type compression tester "SCH" is used. In the tester, the core 4 is placed on a hard plate made of metal. Next, a cylinder made of metal gradually descends toward the core 4. The core 4, squeezed between the bottom face of the cylinder and the hard plate, becomes deformed. A migration distance of the cylinder, starting from the state in which an initial load of 98 N is applied to the core 4 up to the state in which a final load of 1274 N is applied thereto, is measured. A moving speed of the cylinder until the initial

load is applied is 0.83 mm/s. A moving speed of the cylinder after the initial load is applied until the final load is applied is 1.67 mm/s.

The core **4** preferably has a surface hardness K of not less than 65. The core **4** having a surface hardness K of not less than 65 is sufficiently pressed by hold pins in the vicinity of each pole during molding of the cover **6**. By the pressing, a local reduction of the space between the core **4** and a cavity face is suppressed. From this viewpoint, the surface hardness K is more preferably not less than 68 and particularly preferably not less than 70.

The surface hardness K of the core **4** is preferably not greater than 85. When the golf ball **2** having the core **4** having a surface hardness K of not greater than 85 is hit with a putter, soft feel at impact is obtained. From this viewpoint, the surface hardness K is more preferably not greater than 82 and particularly preferably not greater than 80.

The surface hardness K is measured with a Shore C type hardness scale mounted to an automated hardness meter (trade name "digi test II" manufactured by Heinrich Bareiss Prüfgerätebau GmbH). The hardness scale is pressed against the surface of the core **4**. The measurement is conducted in an environment of 23° C.

The ratio (K/S) of the surface hardness K (Shore C) of the core **4** to the amount of compressive deformation S (mm) of the core **4** is preferably not less than 13.0 and not greater than 24.0. In other words, the ratio (K/S) satisfies the following mathematical formula.

$$13.0 \leq K/S \leq 24.0$$

With the core **4** in which the ratio (K/S) is not less than 13.0, a local reduction of the space between the core **4** and the cavity face is suppressed during molding of the cover **6**. The core **4** can contribute to the moldability of the golf ball **2**. From this viewpoint, the ratio (K/S) is more preferably not less than 14.0 and particularly preferably not less than 14.5.

With the core **4** in which the ratio (K/S) is not greater than 24.0, feel at impact upon a shot with a driver and feel at impact upon putting are excellent. From this viewpoint, the ratio (K/S) is more preferably not greater than 23.0 and particularly preferably not greater than 22.5.

The core **4** has a weight of preferably not less than 10 g and not greater than 42 g. The temperature for crosslinking the core **4** is not lower than 140° C. and not higher than 180° C. The time period for crosslinking the core **4** is not shorter than 10 minutes and not longer than 60 minutes.

The cover **6** is positioned outside the core **4**. The cover **6** is the outermost layer excluding the mark layer and the paint layer. The cover **6** is formed from a thermoplastic resin composition. Examples of the base polymer of the resin composition include ionomer resins, thermoplastic polyester elastomers, thermoplastic polyamide elastomers, thermoplastic polyurethane elastomers, thermoplastic polyolefin elastomers, and thermoplastic polystyrene elastomers. Ionomer resins are particularly preferable. Ionomer resins are highly elastic. The golf ball **2** having the cover **6** that includes an ionomer resin has excellent resilience performance. The cover **6** may be formed from a thermosetting resin composition.

An ionomer resin and another resin may be used in combination. In this case, in light of resilience performance, the ionomer resin is included as the principal component of the base polymer. The proportion of the ionomer resin to the entire base polymer is preferably not less than 50% by weight, more preferably not less than 70% by weight, and particularly preferably not less than 85% by weight.

Examples of preferable ionomer resins include binary copolymers formed with an  $\alpha$ -olefin and an  $\alpha,\beta$ -unsaturated carboxylic acid having 3 to 8 carbon atoms. A preferable binary copolymer includes 80% by weight or more but 90% by weight or less of an  $\alpha$ -olefin, and 10% by weight or more but 20% by weight or less of an  $\alpha,\beta$ -unsaturated carboxylic acid. The binary copolymer has excellent resilience performance. Examples of other preferable ionomer resins include ternary copolymers formed with: an  $\alpha$ -olefin; an  $\alpha,\beta$ -unsaturated carboxylic acid having 3 to 8 carbon atoms; and an  $\alpha,\beta$ -unsaturated carboxylate ester having 2 to 22 carbon atoms. A preferable ternary copolymer includes 70% by weight or more but 85% by weight or less of an  $\alpha$ -olefin, 5% by weight or more but 30% by weight or less of an  $\alpha,\beta$ -unsaturated carboxylic acid, and 1% by weight or more but 25% by weight or less of an  $\alpha,\beta$ -unsaturated carboxylate ester. The ternary copolymer has excellent resilience performance. For the binary copolymer and the ternary copolymer, preferable  $\alpha$ -olefins are ethylene and propylene, while preferable  $\alpha,\beta$ -unsaturated carboxylic acids are acrylic acid and methacrylic acid. A particularly preferable ionomer resin is a copolymer formed with ethylene and acrylic acid. Another particularly preferable ionomer resin is a copolymer formed with ethylene and methacrylic acid.

In the binary copolymer and the ternary copolymer, some of the carboxyl groups are neutralized with metal ions. Examples of metal ions for use in neutralization include sodium ion, potassium ion, lithium ion, zinc ion, calcium ion, magnesium ion, aluminum ion, and neodymium ion. The neutralization may be carried out with two or more types of metal ions. Particularly suitable metal ions in light of resilience performance and durability of the golf ball **2** are sodium ion, zinc ion, lithium ion, and magnesium ion.

Specific examples of ionomer resins include trade names "Himilan 1555", "Himilan 1557", "Himilan 1605", "Himilan 1706", "Himilan 1707", "Himilan 1856", "Himilan 1855", "Himilan AM7311", "Himilan AM7315", "Himilan AM7317", "Himilan AM7329", and "Himilan AM7337", manufactured by Du Pont-MITSUI POLYCHEMICALS Co., Ltd.; trade names "Surlyn 6120", "Surlyn 6910", "Surlyn 7930", "Surlyn 7940", "Surlyn 8140", "Surlyn 8150", "Surlyn 8940", "Surlyn 8945", "Surlyn 9120", "Surlyn 9150", "Surlyn 9910", "Surlyn 9945", "Surlyn AD8546", "HPF1000", and "HPF2000", manufactured by E.I. du Pont de Nemours and Company; and trade names "IOTEK 7010", "IOTEK 7030", "IOTEK 7510", "IOTEK 7520", "IOTEK 8000", and "IOTEK 8030", manufactured by ExxonMobil Chemical Corporation. Two or more ionomer resins may be used in combination.

The resin composition of the cover **6** may include a styrene block-containing thermoplastic elastomer. The styrene block-containing thermoplastic elastomer includes a polystyrene block as a hard segment, and a soft segment. A typical soft segment is a diene block. Examples of compounds for the diene block include butadiene, isoprene, 1,3-pentadiene, and 2,3-dimethyl-1,3-butadiene. Butadiene and isoprene are preferable. Two or more compounds may be used in combination.

Examples of styrene block-containing thermoplastic elastomers include styrene-butadiene-styrene block copolymers (SBS), styrene-isoprene-styrene block copolymers (SIS), styrene-isoprene-butadiene-styrene block copolymers (SIBS), hydrogenated SBS, hydrogenated SIS, and hydrogenated SIBS. Examples of hydrogenated SBS include styrene-ethylene-butylene-styrene block copolymers (SEBS). Examples of hydrogenated SIS include styrene-ethylene-propylene-styrene block copolymers (SEPS).

Examples of hydrogenated SIBS include styrene-ethylene-ethylene-propylene-styrene block copolymers (SEEPS).

In light of resilience performance of the golf ball 2, the content of the styrene component in the styrene block-containing thermoplastic elastomer is preferably not less than 10% by weight, more preferably not less than 12% by weight, and particularly preferably not less than 15% by weight. In light of feel at impact of the golf ball 2, the content is preferably not greater than 50% by weight, more preferably not greater than 47% by weight, and particularly preferably not greater than 45% by weight.

In the present invention, styrene block-containing thermoplastic elastomers include an alloy of an olefin and one or more members selected from the group consisting of SBS, SIS, SIBS, SEBS, SEPS, and SEEPS. The olefin component in the alloy is presumed to contribute to improvement of compatibility with another base polymer. The alloy can contribute to the resilience performance of the golf ball 2. An olefin having 2 to 10 carbon atoms is preferable. Examples of suitable olefins include ethylene, propylene, butene, and pentene. Ethylene and propylene are particularly preferable.

Specific examples of polymer alloys include trade names "RABALON T3221C", "RABALON T3339C", "RABALON SJ4400N", "RABALON SJ5400N", "RABALON SJ6400N", "RABALON SJ7400N", "RABALON SJ8400N", "RABALON SJ9400N", and "RABALON SR04", manufactured by Mitsubishi Chemical Corporation. Other specific examples of styrene block-containing thermoplastic elastomers include trade name "Epofriend A1010" manufactured by Daicel Chemical Industries, Ltd., and trade name "SEPTON HG-252" manufactured by Kuray Co., Ltd.

In light of feel at impact upon a shot with a driver and upon putting, the proportion of the styrene block-containing thermoplastic elastomer to the entire base polymer is preferably not less than 2% by weight, more preferably not less than 4% by weight, and particularly preferably not less than 6% by weight. In light of durability, this proportion is preferably not greater than 30% by weight, more preferably not greater than 25% by weight, and particularly preferably not greater than 20% by weight.

The resin composition of the cover 6 may include a coloring agent, a filler, a dispersant, an antioxidant, an ultraviolet absorber, a light stabilizer, a fluorescent material, a fluorescent brightener, and the like in an adequate amount. When the hue of the golf ball 2 is white, a typical coloring agent is titanium dioxide.

The cover 6 preferably has a volume V of not less than 3.0 cm<sup>3</sup>. The cover 6 having a volume V of not less than 3.0 cm<sup>3</sup> can be easily molded. From this viewpoint, the volume V is more preferably not less than 3.5 cm<sup>3</sup> and particularly preferably not less than 3.8 cm<sup>3</sup>.

The volume V of the cover 6 is preferably not greater than 7.0 cm<sup>3</sup>. The golf ball 2 having the cover 6 having a volume V of not greater than 7.0 cm<sup>3</sup> has excellent feel at impact upon a shot with a driver and upon putting. From this viewpoint, the volume V is more preferably not greater than 6.5 cm<sup>3</sup> and particularly preferably not greater than 6.0 cm<sup>3</sup>.

The volume V of the cover 6 can be calculated by the following mathematical formula.

$$V = V_b - V_c - W$$

In this mathematical formula, V<sub>b</sub> represents the volume of the phantom sphere of the golf ball 2, V<sub>c</sub> represents the volume of the core 4, and W represents the total volume of the dimples 8. The meaning of the phantom sphere will be

described in detail later. The meaning of the total volume of the dimples 8 will be described in detail later.

The cover 6 preferably has a hardness H of not greater than 62. The golf ball 2 having the cover 6 having a hardness H of not greater than 62 has excellent feel at impact upon a shot with a driver and upon putting. From this viewpoint, the hardness H is more preferably not greater than 60 and particularly preferably not greater than 58. In light of scuff resistance of the cover 6, the hardness H is preferably not less than 50, more preferably not less than 52, and particularly preferably not less than 54.

The hardness H of the cover 6 is measured according to the standards of "ASTM-D 2240-68". The hardness H is measured with a Shore D type hardness scale mounted to an automated hardness meter (trade name "digi test II" manufactured by Heinrich Bareiss Prüfgerätebau GmbH). For the measurement, a sheet that is formed by hot press, is formed from the same material as that of the cover 6, and has a thickness of about 2 mm, is used. Prior to the measurement, a sheet is kept at 23°C. for two weeks. At the time of measurement, three sheets are stacked.

FIG. 2 is a plan view of the golf ball 2 in FIG. 1, and FIG. 3 is a front view of the golf ball 2. In FIG. 3, an alternate long and two short dashes line Eq indicates an equator, and reference character P indicates poles. Each pole P corresponds to the deepest position of a mold for the golf ball 2. The latitude of the equator Eq is zero. The latitude of each pole P is 90°.

As shown in FIGS. 2 and 3, the contours of most dimples 8 are circular. The golf ball 2 has dimples A each having a diameter of 4.60 mm; dimples B each having a diameter of 4.40 mm; dimples C each having a diameter of 4.30 mm; dimples D each having a diameter of 4.20 mm; dimples E each having a diameter of 4.00 mm; and dimples F each having a diameter of 2.90 mm. The golf ball 2 may have non-circular dimples instead of the circular dimples 8 or together with circular dimples 8. A dimple 8 of which a contour shape is exactly an ellipse is also referred to as a circular dimple 8 in the present invention.

The number of the dimples A is 66; the number of the dimples B is 48; the number of the dimples C is 60; the number of the dimples D is 30; the number of the dimples E is 114; and the number of the dimples F is 12. The total number of the dimples 8 is 330. A dimple pattern is formed by these dimples 8 and the land 10.

FIG. 4 shows a cross section of the golf ball 2 along a plane passing through the central point of the dimple 8 and the central point of the golf ball 2. In FIG. 4, the top-to-bottom direction is the depth direction of the dimple 8. In FIG. 4, an alternate long and two short dashes line 12 indicates a phantom sphere. The surface of the phantom sphere 12 is the surface of the golf ball 2 when it is postulated that no dimple 8 exists. The diameter of the phantom sphere 12 is equal to the diameter of the golf ball 2. The dimple 8 is recessed from the surface of the phantom sphere 12. The land 10 coincides with the surface of the phantom sphere 12. In the present embodiment, the cross-sectional shape of each dimple 8 is substantially a circular arc. The cross-sectional shape may be a curved line of which the curvature changes.

In FIG. 4, an arrow D<sub>m</sub> indicates the diameter of the dimple 8. The diameter D<sub>m</sub> is the distance between two tangent points Ed appearing on a tangent line T<sub>g</sub> that is drawn tangent to the far opposite ends of the dimple 8. Each tangent point Ed is also the edge of the dimple 8. The edge Ed defines the contour of the dimple 8. In FIG. 4, a double ended arrow D<sub>p</sub> indicates the depth of the dimple 8. The

## 11

depth  $D_p$  is the distance between the deepest point of the dimple **8** and the surface of the phantom sphere **12**.

The diameter  $D_m$  of each dimple **8** is preferably not less than 2.0 mm and not greater than 6.0 mm. The dimple **8** having a diameter  $D_m$  of not less than 2.0 mm disturbs the air flow around the golf ball **2** when the golf ball **2** flies. This phenomenon is referred to as turbulization. Owing to the turbulization, a large flight distance of the golf ball **2** is achieved. From this viewpoint, the diameter  $D_m$  is more preferably not less than 2.5 mm and particularly preferably not less than 2.8 mm. The dimple **8** having a diameter  $D_m$  of not greater than 6.0 mm does not impair a fundamental feature of the golf ball **2** being substantially a sphere. From this viewpoint, the diameter  $D_m$  is more preferably not greater than 5.5 mm and particularly preferably not greater than 5.0 mm.

The area  $A_r$  of the dimple **8** is the area of a region surrounded by the contour line of the dimple **8** when the central point of the golf ball **2** is viewed at infinity. In the case of a circular dimple **8**, the area  $A_r$  is calculated by the following mathematical formula.

$$A_r = (D_m/2)^2 * \pi$$

In the golf ball **2** shown in FIGS. 2 and 3, the area  $A_r$  of each dimple A is 16.6 mm<sup>2</sup>; the area  $A_r$  of each dimple B is 15.2 mm<sup>2</sup>; the area  $A_r$  of each dimple C is 14.5 mm<sup>2</sup>; the area  $A_r$  of each dimple D is 13.9 mm<sup>2</sup>; the area  $A_r$  of each dimple E is 12.6 mm<sup>2</sup>; and the area  $A_r$  of each dimple F is 6.6 mm<sup>2</sup>.

In the present specification, the ratio of the sum of the areas  $A_r$  of all the dimples **8** relative to the surface area of the phantom sphere **12** is referred to as an occupation ratio. From the viewpoint of achieving sufficient turbulization, the occupation ratio is preferably not less than 78%, more preferably not less than 80%, and particularly preferably not less than 82%. The occupation ratio is preferably not greater than 95%.

In light of suppression of rising of the golf ball **2** during flight, the depth  $D_p$  of each dimple **8** is preferably not less than 0.10 mm, more preferably not less than 0.15 mm, and particularly preferably not less than 0.17 mm. In light of suppression of dropping of the golf ball **2** during flight, the depth  $D_p$  is preferably not greater than 0.60 mm, more preferably not greater than 0.50 mm, and particularly preferably not greater than 0.40 mm.

In the present invention, the "volume of the dimple" means the volume of a portion surrounded by the surface of the phantom sphere **12** and the dimple **8**. The total volume  $W$  of the dimples **8** is preferably not less than 490 mm<sup>3</sup> and not greater than 620 mm<sup>3</sup>. With the golf ball **2** having a total volume  $W$  of not less than 490 mm<sup>3</sup>, rising of the golf ball **2** during flight is suppressed. From this viewpoint, the total volume  $W$  is more preferably not less than 520 mm<sup>3</sup> and particularly preferably not less than 530 mm<sup>3</sup>. With the golf ball **2** having a total volume  $W$  of not greater than 620 mm<sup>3</sup>, dropping of the golf ball **2** during flight is suppressed. From this viewpoint, the total volume  $W$  is more preferably not greater than 600 mm<sup>3</sup> and particularly preferably not greater than 580 mm<sup>3</sup>.

The number of the dimples **8** is preferably not less than 300 and not greater than 400. In a mold for the golf ball **2** in which the number of the dimples **8** is in this range, the thicknesses of support pins, described in detail later, are appropriate. From this viewpoint, the number of the dimples **8** is more preferably not less than 310 and not greater than 390, and particularly preferably not less than 320 and not greater than 380.

## 12

FIG. 5 shows a mold **14** for the golf ball **2** in FIG. 1. The mold **14** is used for injection molding. In FIG. 5, the core **4** is also shown. The mold **14** has an upper mold half **16** and a lower mold half **18**. When the upper mold half **16** and the lower mold half **18** are mated with each other, a cavity is formed. The mold **14** has a cavity face **20**.

A parting line **PL** between the upper mold half **16** and the lower mold half **18** corresponds to the equator **Eq** of the golf ball **2**. The parting line **PL** may be slightly displaced from the equator **Eq**. The parting line **PL** may have a zigzag shape. A plurality of gates **22** are present on the parting line **PL**. These gates **22** are aligned along the equator of the cavity. The gates **22** may be slightly displaced from the equator. The latitude of an opening of each gate **22** that is formed in the cavity face **20** is preferably not less than 0° and not greater than 20°. In the mold **14** shown in FIG. 5, this latitude is zero.

The upper mold half **16** has a plurality of pin holes **24** and a plurality of support pins **26**. Each support pin **26** is passed through the pin hole **24**. The support pins **26** can advance in the downward direction in FIG. 5. The support pins **26** can retract in the upward direction in FIG. 5.

The lower mold half **18** has a plurality of pin holes **24** and a plurality of support pins **26**. Each support pin **26** is passed through the pin hole **24**. The support pins **26** can advance in the upward direction in FIG. 5. The support pins **26** can retract in the downward direction in FIG. 5.

The core **4** is placed into the mold **14**, and the upper mold half **16** and the lower mold half **18** are mated with each other. The support pins **26** move toward the core **4**, and leading ends of the support pins **26** come into contact with the core **4**. The core **4** is held at the center of the cavity by these support pins **26**. A state where the core **4** is held is shown in FIG. 5. A melted resin composition is injected through the gates **22** toward the space between the cavity face **20** and the core **4**. The resin composition flows toward the poles of the cavity. Immediately before the injection of the resin composition is completed, the support pins **26** retract. Each support pin **26** retracts to a position at which the leading end thereof substantially coincides with the cavity face **20**. Spaces formed as a result of the retraction of the support pins **26** are also filled with the resin composition. The resin composition becomes solidified, whereby the cover **6** is formed. In FIG. 6, the mold **14** immediately after the formation of the cover **6** is completed is shown.

FIG. 7 is a partially enlarged view of the mold **14** in FIG. 6 with the core **4** and the cover **6**. In FIG. 7, the lower mold half **18** is shown. The upper mold half **16** has a shape that is obtained by vertically inverting the shape shown in FIG. 5. The cavity face **20** of the mold **14** has a large number of first pimples **28**. Dimples **8** are formed at portions of the surface of the cover **6** that are in contact with the respective first pimples **28**. The dimples **8** have a shape that is the inverted shape of the first pimples **28**.

As shown in FIG. 7, the support pin **26** has a second pimple **30** at the leading end thereof. Dimples **8** are formed at portions of the surface of the cover **6** that are in contact with the respective second pimples **30**. The dimples **8** have a shape that is the inverted shape of the second pimples **30**. In the case where a cross-section of the support pin **26** that is perpendicular to the axial direction thereof has a circular shape, the contour of the second pimple **30** is substantially an ellipse. Therefore, the shape of the dimple **8** that is in contact with the second pimple **30** is not exactly a circle but an ellipse. In the present invention, this elliptical dimple **8** is also referred to as a "circular dimple". One support pin **26** may have two second pimples **30**.

The dimples 8 that are not hatched in FIGS. 2 and 3 are formed by the first pimples 28. The dimples 8 that are hatched in FIGS. 2 and 3 are formed by the second pimples 30. The golf ball 2 has: six dimples 8 formed by the second pimples 30 of the upper mold half 16; and six dimples 8 formed by the second pimples 30 of the lower mold half 18. In other words, the mold 14 has six support pins 26 in the upper mold half 16 and six support pins 26 in the lower mold half 18. Therefore, the number of the support pins 26 is twelve. The golf ball 2 has twelve dimples 8 that are formed by the second pimples 30.

Due to the pressure of the melted resin composition that has passed through the gates 22, the core 4 is reduced radially in the right-left direction in FIG. 5 and enlarged radially in the top-to-bottom direction in FIG. 5. Due to this deformation, in the vicinity of each pole P (see FIG. 3), the space between the core 4 and the cavity face 20 is reduced. This reduction may cause a failure of injection of the resin composition to the vicinity of each pole P. By the support pins 26 sufficiently pressing the core 4, deformation of the core 4 is suppressed, and a failure of injection of the resin composition is suppressed.

The number of the support pins 26 is preferably not less than 8 and not greater than 12. With the mold 14 in which this number is not less than 8, deformation of the core 4 can be suppressed during molding of the cover 6. The structure of the mold 14 in which this number is not greater than 12 is simple. In addition, with the mold 14 in which this number is not greater than 12, the golf ball 2 having excellent appearance can be produced.

FIG. 8 is a partially enlarged view of the support pin 26 of the mold 14 in FIG. 7. In FIG. 8, reference character P1 indicates a point in the second pimple 30 that is closest to the pole, and reference character P2 indicates a point in the second pimple 30 that is closest to the equator. Reference character Pc indicates the midpoint of a straight line connecting the point P1 and the point P2. Reference character L1 indicates a straight line passing through the midpoint Pc and the center of the cavity (not shown). An arrow  $\alpha$  indicates the angle between the straight line L1 and the horizontal direction. The angle  $\alpha$  is also the latitude of the point Pc. In the present invention, the angle  $\alpha$  is referred to as a "latitude of the support pin".

The latitude  $\alpha$  is preferably not less than 65°. Deformation of the core 4 due to the injection pressure for the cover 6 is suppressed by each support pin 26 having a latitude  $\alpha$  of not less than 65°. By this support pin 26, a sufficient space is maintained between the core 4 and the cavity face 20 during molding of the cover 6. By this support pin 26, a failure of injection for the cover 6 can be suppressed. From this viewpoint, the latitude  $\alpha$  is more preferably not less than 70° and particularly preferably not less than 72°.

From the viewpoint that the core 4 is stably held by the support pins 26 and from the viewpoint that the mold 14 is easily produced, the latitude  $\alpha$  is preferably not greater than 85°, more preferably not greater than 83°, and particularly preferably not greater than 81°.

The product ( $\alpha^*V$ ) of the latitude  $\alpha$  (degree) of each support pin 26 and the volume V (cm<sup>3</sup>) of the cover 6 is preferably not less than 300. When the product ( $\alpha^*V$ ) is not less than 300, a failure of injection for the cover 6 in the vicinity of each pole P can be suppressed. From this viewpoint, the product ( $\alpha^*V$ ) is more preferably not less than 335 and particularly preferably not less than 370. The product ( $\alpha^*V$ ) is preferably not greater than 550, more preferably not greater than 515, and particularly preferably not greater than 480.

## EXAMPLES

## Example 1

5 A rubber composition a was obtained by kneading 100 parts by weight of a high-cis polybutadiene (trade name "BR-730", manufactured by JSR Corporation), 27.4 parts by weight of zinc diacrylate, 5 parts by weight of zinc oxide, an appropriate amount of barium sulfate, 0.5 parts by weight of diphenyl disulfide, and 0.9 parts by weight of dicumyl peroxide. This rubber composition a was placed into a mold including upper and lower mold halves each having a hemispherical cavity, and heated at 160° C. for 20 minutes to obtain a core with a diameter of 40.5 mm. The amount of barium sulfate was adjusted such that a core having an appropriate weight was obtained.

10 A resin composition #1 was obtained by kneading 47 parts by weight of an ionomer resin (the aforementioned "Himilan 1555"), 46 parts by weight of another ionomer resin (the aforementioned "Himilan 1557"), 7 parts by weight of a styrene block-containing thermoplastic elastomer (the aforementioned "Rabalon T3221C"), 4 parts by weight of titanium dioxide, and 0.2 parts by weight of a light stabilizer (trade name "JF-90", manufactured by Johoku Chemical Co., Ltd.) with a twin-screw kneading extruder. The mold 15 shown in FIGS. 5 to 8 was prepared. The mold has 12 support pins. The latitude  $\alpha$  of each support pin is 72.5°. The core was placed into the mold. The melted resin composition #1 was injected so as to cover the core to form a cover. The thickness of the cover was 1.1 mm. Dimples having a shape that is the inverted shape of the pimples were formed on the cover.

20 A clear paint including a two-component curing type polyurethane as a base material was applied to this cover to obtain a golf ball of Example 1 with a diameter of about 42.7 mm and a weight of about 45.6 g. The dimple pattern of the golf ball and the positions of the support pins are shown in FIGS. 2 and 3. Specifications (i) of the dimples of the golf ball are shown in detail in Table 3 below.

## Examples 2 to 10 and Comparative Examples 1 to 6

35 Golf balls of Examples 2 to 10 and Comparative Examples 1 to 6 were obtained in the same manner as Example 1, except the specifications of the core, the cover, and the dimples were as shown in Tables 4 to 8 below. The composition of the core is shown in detail in Tables 1 and 2 below. The composition of the cover is shown in detail in Table 3 below. The specifications of the dimples are shown in detail in Table 4 below.

40 [Flight Test]  
50 A driver (trade name "XXIO", manufactured by DUNLOP SPORTS CO. LTD., shaft hardness: R, loft angle: 10.5°) was attached to a swing machine manufactured by Golf Laboratories, Inc. A golf ball was hit under a condition of a head speed of 40 m/sec, and the flight distance was measured. The flight distance is the distance between the point at the hit and the point at which the golf ball stopped. The average of values obtained by 12 measurements is shown in Tables 4 to 8 below.

## [Feel at Impact Upon Shot with Driver]

55 Thirty golf players hit golf balls with drivers and were asked about feel at impact. The evaluation was categorized as follows on the basis of the number of golf players who answered, "The feel at impact was favorable".

A: 25 persons or more

B: 20 to 24 persons

C: 15 to 19 persons

D: 14 persons or less

60 65 The results are shown in Tables 4 to 8 below.

## [Feel at Impact Upon Putting]

Thirty golf players hit golf balls with putters and were asked about feel at impact. The evaluation was categorized as follows on the basis of the number of golf players who answered, "The feel at impact was favorable".

- A: 25 persons or more
- B: 20 to 24 persons
- C: 15 to 19 persons
- D: 14 persons or less

The results are shown in Tables 4 to 8 below.

## [Moldability]

120 golf balls were molded by injection molding. The evaluation was categorized as follows on the basis of the number of golf balls for which a molding failure occurred. A molding failure means a state where a part of the surface of the core is not covered with the resin composition of the cover.

- A: 0
- B: 1
- C: 2
- D: 3 or more

The results are shown in Tables 4 to 8 below.

TABLE 1

| Composition of Core (parts by weight) |      |      |      |      |
|---------------------------------------|------|------|------|------|
| Rubber composition                    |      |      |      |      |
|                                       | a    | b    | c    | d    |
| Polybutadiene rubber BR-730           | 100  | 100  | 100  | 100  |
| Zinc diacrylate                       | 27.4 | 25.4 | 19.4 | 31.6 |
| Zinc oxide                            | 5    | 5    | 5    | 5    |
| Barium sulfate                        | AA   | AA   | AA   | AA   |
| Benzoic acid                          | —    | —    | —    | 2    |
| DPDS                                  | 0.5  | 0.5  | 0.5  | 0.5  |
| Dicumyl peroxide                      | 0.9  | 0.9  | 0.9  | 0.9  |

AA: Appropriate amount

TABLE 2

| Composition of Core (parts by weight) |      |      |      |
|---------------------------------------|------|------|------|
| Rubber composition                    |      |      |      |
|                                       | e    | f    | g    |
| Polybutadiene rubber BR-730           | 100  | 100  | 100  |
| Zinc diacrylate                       | 24.7 | 21.2 | 17.8 |
| Zinc oxide                            | 5    | 5    | 5    |
| Barium sulfate                        | AA   | AA   | AA   |
| Benzoic acid                          | 2    | 2    | 2    |
| DPDS                                  | 0.5  | 0.5  | 0.5  |
| Dicumyl peroxide                      | 0.9  | 0.9  | 0.9  |

AA: Appropriate amount

TABLE 3

| Composition of Cover (parts by weight) |    |    |    |
|----------------------------------------|----|----|----|
| Resin composition                      |    |    |    |
|                                        | 1  | 2  | 3  |
| Himilan AM7337                         | —  | —  | —  |
| Himilan AM7329                         | —  | 40 | 63 |
| Himilan 1555                           | 47 | —  | 35 |
| Himilan 1557                           | 46 | —  | —  |
| Himilan 1605                           | —  | 54 | —  |

TABLE 3-continued

| Composition of Cover (parts by weight) |                               |     |     |     |   |
|----------------------------------------|-------------------------------|-----|-----|-----|---|
| 5                                      | Resin composition             |     |     |     |   |
|                                        | 1                             | 2   | 3   | 4   | 5 |
| 10                                     | Rabalon T3221C                | 7   | 6   | 2   |   |
|                                        | Titanium dioxide (A220)       | 4   | 3   | 3   |   |
|                                        | JF-90                         | 0.2 | 0.2 | 0.2 |   |
|                                        | Slab hardness<br>(D hardness) | 57  | 60  | 63  |   |
|                                        |                               |     |     |     |   |

TABLE 4

| Specifications of Dimples |      |        |            |            |            |                              |
|---------------------------|------|--------|------------|------------|------------|------------------------------|
| 20                        | Type | Number | Dm<br>(mm) | Dp<br>(mm) | CR<br>(mm) | Volume<br>(mm <sup>3</sup> ) |
| 25                        | i    | 66     | 4.60       | 0.264      | 19.0       | 2.198                        |
|                           |      | 48     | 4.40       | 0.254      | 17.4       | 1.931                        |
|                           |      | 60     | 4.30       | 0.249      | 16.6       | 1.807                        |
|                           |      | 30     | 4.20       | 0.244      | 15.8       | 1.689                        |
|                           |      | 114    | 4.00       | 0.229      | 14.9       | 1.440                        |
|                           | ii   | 12     | 2.90       | 0.179      | 8.2        | 0.593                        |
|                           |      | 66     | 4.60       | 0.229      | 25.2       | 1.907                        |
|                           |      | 48     | 4.40       | 0.219      | 23.1       | 1.664                        |
|                           |      | 60     | 4.30       | 0.214      | 22.1       | 1.552                        |
|                           |      | 30     | 4.20       | 0.209      | 21.1       | 1.446                        |
|                           | iii  | 114    | 4.00       | 0.194      | 20.1       | 1.219                        |
|                           |      | 12     | 2.90       | 0.144      | 11.1       | 0.477                        |
|                           |      | 66     | 4.60       | 0.289      | 16.1       | 2.407                        |
|                           |      | 48     | 4.40       | 0.279      | 14.7       | 2.122                        |
|                           |      | 60     | 4.30       | 0.274      | 14.1       | 1.989                        |
|                           |      | 30     | 4.20       | 0.269      | 13.4       | 1.863                        |
|                           |      | 114    | 4.00       | 0.254      | 12.6       | 1.598                        |
|                           |      | 12     | 2.90       | 0.204      | 6.9        | 0.677                        |
|                           |      | 168    | 4.50       | 0.275      | 16.3       | 2.189                        |
|                           |      | 168    | 3.40       | 0.214      | 10.0       | 0.972                        |
| 35                        | iv   | 30     | 4.40       | 0.254      | 17.4       | 1.931                        |
|                           |      | 140    | 4.30       | 0.249      | 16.6       | 1.807                        |
|                           |      | 90     | 4.20       | 0.244      | 15.8       | 1.689                        |
|                           |      | 40     | 3.95       | 0.227      | 14.5       | 1.390                        |
|                           |      | 40     | 3.50       | 0.202      | 11.8       | 0.972                        |
| 40                        | v    | 168    | 4.50       | 0.275      | 16.3       | 2.189                        |
|                           |      | 168    | 3.40       | 0.214      | 10.0       | 0.972                        |
|                           |      | 30     | 4.40       | 0.254      | 17.4       | 1.931                        |
|                           |      | 140    | 4.30       | 0.249      | 16.6       | 1.807                        |
|                           |      | 90     | 4.20       | 0.244      | 15.8       | 1.689                        |

TABLE 5

| Results of Evaluation |                             |                             |           |           |           |
|-----------------------|-----------------------------|-----------------------------|-----------|-----------|-----------|
| 50                    | Core                        | Comp.                       | Example 1 | Example 2 | Example 3 |
| Composition           | d                           | a                           | b         | c         | e         |
| Diameter (mm)         | 40.5                        | 40.5                        | 40.5      | 40.5      | 40.5      |
| Deformation S (mm)    | 3.5                         | 3.5                         | 4.0       | 4.5       |           |
| K (Shore C)           | 87                          | 79                          | 76        | 79        |           |
| 55                    | Cover                       | Composition                 | 1         | 1         | 1         |
|                       |                             | Thickness (mm)              | 1.1       | 1.1       | 1.1       |
|                       |                             | H (Shore D)                 | 57        | 57        | 57        |
|                       |                             | Volume V (cm <sup>3</sup> ) | 5.41      | 5.41      | 5.41      |
|                       |                             | Dimples                     |           |           |           |
| 60                    | Pattern                     | I                           | I         | I         | I         |
|                       |                             | Plan view                   | FIG. 2    | FIG. 2    | FIG. 2    |
|                       |                             | Front view                  | FIG. 3    | FIG. 3    | FIG. 3    |
|                       |                             | Total number                | 330       | 330       | 330       |
|                       |                             | Specifications              | i         | i         | i         |
| 65                    | Volume W (mm <sup>3</sup> ) | 568                         | 568       | 568       | 568       |

TABLE 5-continued

| Results of Evaluation      |                    |           |           |           |
|----------------------------|--------------------|-----------|-----------|-----------|
|                            | Comp.<br>Example 1 | Example 1 | Example 2 | Example 3 |
| <u>Support pins</u>        |                    |           |           |           |
| $\alpha$ (deg.)            | 72.5               | 72.5      | 72.5      | 72.5      |
| Number                     | 12                 | 12        | 12        | 12        |
| K/S                        | 24.9               | 22.6      | 19.0      | 17.6      |
| $\alpha * V$               | 392                | 392       | 392       | 392       |
| Flight distance<br>(index) | 97                 | 98        | 99        | 100       |
| Feeling W#1                | C                  | C         | B         | B         |
| Feeling putter             | D                  | C         | B         | C         |
| Moldability                | A                  | A         | A         | A         |

TABLE 6

| Results of Evaluation |                    |           |                    |                    |
|-----------------------|--------------------|-----------|--------------------|--------------------|
|                       | Comp.<br>Example 4 | Example 5 | Comp.<br>Example 2 | Comp.<br>Example 3 |

|                             |        |        |        |         |
|-----------------------------|--------|--------|--------|---------|
| <u>Core</u>                 |        |        |        |         |
| Composition                 | f      | g      | c      | e       |
| Diameter (mm)               | 40.5   | 40.5   | 40.5   | 41.1    |
| Deformation S (mm)          | 5.0    | 5.5    | 5.5    | 4.5     |
| K (Shore C)                 | 76     | 72     | 69     | 80      |
| <u>Cover</u>                |        |        |        |         |
| Composition                 | 1      | 1      | 1      | 1       |
| Thickness (mm)              | 1.1    | 1.1    | 1.1    | 0.8     |
| H (Shore D)                 | 57     | 57     | 57     | 57      |
| Volume V (cm <sup>3</sup> ) | 5.41   | 5.41   | 5.41   | 3.86    |
| <u>Dimples</u>              |        |        |        |         |
| Pattern                     | I      | I      | I      | V       |
| Plan view                   | FIG. 2 | FIG. 2 | FIG. 2 | FIG. 15 |
| Front view                  | FIG. 3 | FIG. 3 | FIG. 3 | FIG. 16 |
| Total number                | 330    | 330    | 330    | 340     |
| Specifications              | i      | i      | i      | v       |
| Volume W (mm <sup>3</sup> ) | 568    | 568    | 568    | 557     |
| <u>Support pins</u>         |        |        |        |         |

|                            |      |      |      |      |
|----------------------------|------|------|------|------|
| $\alpha$ (deg.)            | 72.5 | 72.5 | 72.5 | 74.6 |
| Number                     | 12   | 12   | 12   | 10   |
| K/S                        | 15.2 | 13.1 | 12.5 | 17.8 |
| $\alpha * V$               | 392  | 392  | 392  | 288  |
| Flight distance<br>(index) | 100  | 101  | 100  | 101  |
| Feeling W#1                | A    | A    | A    | B    |
| Feeling putter             | B    | A    | A    | C    |
| Moldability                | A    | B    | D    | D    |

TABLE 7

| Results of Evaluation |           |           |           |           |
|-----------------------|-----------|-----------|-----------|-----------|
|                       | Example 6 | Example 7 | Example 8 | Example 9 |

|                             |      |      |      |      |
|-----------------------------|------|------|------|------|
| <u>Core</u>                 |      |      |      |      |
| Composition                 | e    | f    | g    | f    |
| Diameter (mm)               | 41.1 | 40.5 | 40.5 | 39.9 |
| Deformation S (mm)          | 4.5  | 5.0  | 5.5  | 5.0  |
| K (Shore C)                 | 80   | 76   | 72   | 75   |
| <u>Cover</u>                |      |      |      |      |
| Composition                 | 1    | 1    | 1    | 1    |
| Thickness (mm)              | 0.8  | 1.1  | 1.1  | 1.4  |
| H (Shore D)                 | 57   | 57   | 57   | 57   |
| Volume V (cm <sup>3</sup> ) | 3.86 | 5.45 | 5.45 | 6.95 |

TABLE 7-continued

| Results of Evaluation |           |           |           |           |
|-----------------------|-----------|-----------|-----------|-----------|
|                       | Example 6 | Example 7 | Example 8 | Example 9 |

|    |                             |         |         |         |         |
|----|-----------------------------|---------|---------|---------|---------|
| 5  | <u>Dimples</u>              |         |         |         |         |
| 10 | Pattern                     | IV      | III     | II      | V       |
|    | Plan view                   | FIG. 13 | FIG. 11 | FIG. 9  | FIG. 15 |
|    | Front view                  | FIG. 14 | FIG. 12 | FIG. 10 | FIG. 16 |
|    | Total number                | 340     | 336     | 336     | 340     |
|    | Specifications              | v       | iv      | iv      | v       |
|    | Volume W (mm <sup>3</sup> ) | 557     | 531     | 531     | 557     |
|    | Support pins                |         |         |         |         |

|    |                            |      |      |      |      |
|----|----------------------------|------|------|------|------|
| 15 | <u>Core</u>                |      |      |      |      |
| 20 | $\alpha$ (deg.)            | 81.9 | 67.5 | 80.9 | 74.6 |
|    | Number                     | 10   | 8    | 8    | 10   |
|    | K/S                        | 17.8 | 15.2 | 13.1 | 15.0 |
|    | $\alpha * V$               | 316  | 368  | 441  | 518  |
|    | Flight distance<br>(index) | 101  | 97   | 98   | 102  |
|    | Feeling W#1                | B    | A    | A    | A    |
|    | Feeling putter             | C    | B    | A    | B    |
|    | Moldability                | B    | B    | B    | C    |

| Results of Evaluation |                    |                    |                     |                    |
|-----------------------|--------------------|--------------------|---------------------|--------------------|
|                       | Comp.<br>Example 4 | Comp.<br>Example 5 | Comp.<br>Example 10 | Comp.<br>Example 6 |

|    |                    |      |      |      |      |
|----|--------------------|------|------|------|------|
| 25 | <u>Core</u>        |      |      |      |      |
| 30 | Composition        | e    | e    | e    | e    |
|    | Diameter (mm)      | 40.5 | 40.5 | 40.5 | 40.5 |
|    | Deformation S (mm) | 4.5  | 4.5  | 4.5  | 4.5  |
|    | K (Shore C)        | 79   | 79   | 79   | 79   |
|    | Cover              |      |      |      |      |

|    |                             |      |      |      |      |
|----|-----------------------------|------|------|------|------|
| 35 | <u>Dimples</u>              |      |      |      |      |
| 40 | Composition                 | 1    | 1    | 2    | 3    |
|    | Thickness (mm)              | 1.1  | 1.1  | 1.1  | 1.1  |
|    | H (Shore D)                 | 57   | 57   | 60   | 63   |
|    | Volume V (cm <sup>3</sup> ) | 5.49 | 5.36 | 5.41 | 5.41 |
|    | Support pins                |      |      |      |      |

|    |                             |        |        |        |        |
|----|-----------------------------|--------|--------|--------|--------|
| 45 | <u>Core</u>                 |        |        |        |        |
| 50 | Composition                 | I      | I      | I      | I      |
|    | Plan view                   | FIG. 2 | FIG. 2 | FIG. 2 | FIG. 2 |
|    | Front view                  | FIG. 3 | FIG. 3 | FIG. 3 | FIG. 3 |
|    | Total number                | 330    | 330    | 330    | 330    |
|    | Specifications              | ii     | iii    | i      | i      |
|    | Volume W (mm <sup>3</sup> ) | 487    | 626    | 568    | 568    |
|    | Support pins                |        |        |        |        |

|    |                            |      |      |      |      |
|----|----------------------------|------|------|------|------|
| 55 | <u>Core</u>                |      |      |      |      |
| 60 | $\alpha$ (deg.)            | 72.5 | 72.5 | 72.5 | 72.5 |
|    | Number                     | 12   | 12   | 12   | 12   |
|    | K/S                        | 17.6 | 17.6 | 17.6 | 17.6 |
|    | $\alpha * V$               | 398  | 388  | 392  | 392  |
|    | Flight distance<br>(index) | 95   | 95   | 101  | 102  |
|    | Feeling W#1                | B    | B    | C    | D    |
|    | Feeling putter             | C    | C    | C    | D    |
|    | Moldability                | A    | A    | A    | A    |

As shown in Tables 4 to 8, the golf ball of each Example is excellent in various performance characteristics. From the evaluation results, advantages of the present invention are clear.

The golf ball according to the present invention is suitable for, for example, playing golf on golf courses and practicing at driving ranges. The above descriptions are merely illustrative examples, and various modifications can be made without departing from the principles of the present invention.

## 19

What is claimed is:

1. A golf ball comprising a core and a cover positioned outside the core and molded in a mold having a plurality of support pins by injection molding, wherein a ratio (K/S) of a surface hardness K (Shore C) of the core

to an amount of compressive deformation S (mm) of the core satisfies the following mathematical formula,

$$14.5 \leq K/S \leq 22.5,$$

the cover has a hardness H (Shore D) of not greater than 58,

the golf ball has a plurality of dimples on a surface thereof,

a total volume W of the dimples is not less than 490 mm<sup>3</sup> and not greater than 620 mm<sup>3</sup>, and

a product ( $\alpha^*V$ ) of a latitude  $\alpha$  (degree) of each support pin and a volume V (cm<sup>3</sup>) of the cover is not less than 370 and not greater than 480,

the surface hardness K is not less than 70 Shore C, the amount of compressive deformation S is not less than 4.0 mm, and

the cover volume V is not less than 3.8 cm<sup>3</sup> and not greater than 6.0 cm<sup>3</sup>.

2. The golf ball according to claim 1, wherein a number of the support pins is not less than 8 and not greater than 12.

3. The golf ball according to claim 1, wherein a number of the dimples is not less than 300 and not greater than 400.

4. The golf ball according to claim 1, wherein the golf ball has a two-piece structure.

## 20

5. A method for producing a golf ball, the method comprising the steps of:

placing a core into a mold having a plurality of support pins and having a cavity face including a plurality of pimples;

holding the core in a cavity of the mold by the support pins;

injecting a melted resin composition into a space between the cavity face and the core; and

solidifying the resin composition to mold a cover and form a plurality of dimples having a shape that is an inverted shape of the pimples, wherein

a ratio (K/S) of a surface hardness K (Shore C) of the core to an amount of compressive deformation S (mm) of the core satisfies the following mathematical formula,

$$14.5 \leq K/S \leq 22.5,$$

the cover has a Shore D hardness of not greater than 58, a total volume W of the dimples is not less than 490 mm<sup>3</sup> and not greater than 620 mm<sup>3</sup>, and

a product ( $\alpha^*V$ ) of a latitude  $\alpha$  (degree) of each support pin and a volume V (cm<sup>3</sup>) of the cover is not less than 370 and not greater than 480,

the surface hardness K is not less than 70 Shore C, the amount of compressive deformation S is not less than 4.0 mm, and

a volume V of the cover is not less than 3.8 cm<sup>3</sup> and not greater than 6.0 cm<sup>3</sup>.

\* \* \* \* \*